

June 16, 1942.

R. S. DEAN

2,286,199

MANGANESE ALLOY

Filed July 16, 1938



Inventor  
Reginald S. Dean.  
By McLaughlin and Hallenstein  
Atty's.

## UNITED STATES PATENT OFFICE

2,286,199

## MANGANESE ALLOY

Reginald S. Dean, Washington, D. C., assignor to  
Chicago Development Company, Chicago, Ill.

Application July 16, 1938, Serial No. 219,501

1 Claim. (CL 75—126)

My present invention relates to alloys containing manganese, iron and chromium, and is filed as a continuation-in-part of my prior copending application Serial No. 199,329, filed April 1, 1938.

My present invention may be considered from several aspects, depending upon the characteristics, properties and constitution of the alloys coming within the range to which my invention relates. As an example, it may be pointed out that so-called stainless steels of the type containing 18% chromium, 8% nickel and balance iron are not usable for all purposes. Where a considerable degree of hardness is desired, this type of alloy cannot be used. If sufficient amounts of carbon are introduced, and the alloy is appropriately heat treated, a substantial hardening will result, but the stainless properties are concomitantly lost. So-called stainless steels of this type are objectionable also in containing a relatively expensive ingredient, namely nickel, which is required to maintain the austenitic character of the alloy to which, in part at least, is attributable its stainless properties. Attempts have been made to substitute manganese in whole or in part for the nickel in this type of alloy, and it is well known that alloys of manganese, chromium and iron are much more resistant to sulfur-containing gases and other forms of corrosion than other alloys which have been used for the purpose. They seem to offer certain advantages over the 18-8 types of alloys, but attempts to make truly stainless alloys of this character have not been satisfactory, particularly where other desirable properties must be retained. For example, it was found that the chromium content could not be raised sufficiently to prevent scaling above 800 degrees C. without the introduction of extreme brittleness. It has generally been accepted that in manganese-iron-chromium alloys containing 30% manganese or more, not more than 10 or 11% of chromium can be present without producing such extreme brittleness as to result in the alloy being substantially worthless for any useful purpose. This brittleness was supposed to be due to the formation of the compound FeCr. Even with lower amounts of manganese, such as 15%, the prior art found it impossible to introduce more than approximately 15% of chromium without the occurrence of brittleness. These considerations are introduced entirely by way of illustration, and are adequate to show the problems which the prior art faces in attempting to produce alloys of manganese, iron and chromium having properties which would make them suitable for employment in the same general fields in which other types of ferrous alloys, stainless and otherwise, are customarily employed.

I have found that by employing certain concentrations of iron, chromium and manganese, I can produce alloys of very remarkable properties,

some of the important characteristics of which will be explained hereinafter, and I have found also that these properties are particularly obtainable within the range which I have established by the utilization of substantially pure manganese such as that prepared by the electrolytic process as described in the U. S. Bureau of Mines Report of Investigations, No. 3322, or substantially pure manganese made by other methods but approximating the product identified in purity. This manganese has the following typical composition: Fe, .007%; Si, .001%; Pb, .002%; Zn, .001%; Mo, .001%; Sn, .0005%; Cu, .0005%; Ni, .0005%; Co, .0005%; Ag, .0001%; As+Sb, .0001%; total Ti, Al, Zr, Cr, V, U, Be, Ta, Cb, P, and rare earths, .001%; S, total, 0.276%; S, as sulphide, .17%; Mn, 99.7088%.

Manganese of this general typical composition may also be prepared by the distillation of commercially pure manganese and by the utilization of modified electrolytic processes, the nature of which need not be set out for a full understanding of the present invention.

By the use of manganese of high purity and by means of appropriate treatment for desulphurization, such as treatment with calcium carbide, metallic calcium and other agents, I have found it possible to produce ductile alloys having a composition up to about 17% chromium and 35% manganese with the balance substantially iron. Such alloys are malleable at elevated temperature, such as at 1200 degrees C., and, by cooling from this temperature to a temperature of 750 degrees C. and maintaining them at this temperature for several hours, a permanently ductile alloy is obtained having great resistance to corrosion by sulphur-containing gases at elevated temperatures.

Within the range which I have discovered, I have found it possible to produce hardenable stainless alloys, wherein there is a considerable range of ductility, a considerable range of hardening properties both through heat treatment and cold work, and a range of stainless properties, all as will be described hereinafter, enabling those skilled in the art to utilize iron-manganese-chromium alloys in a way and for purposes which, as far as I know, have been impossible so far as prior art disclosures are concerned.

My invention may be considered with the accompanying drawing, in which

Fig. 1 is a ternary diagram on a relatively small scale, indicating the general range in which the alloys of my present invention are found; and

Fig. 2 is a fragmentary portion of the ternary diagram of Fig. 1, with the iron scale shown in a modified position, this diagram being of sufficient size so that the characteristics and properties of the various alloys may be readily deter-

mined from a consideration of such diagram and the description which accompanies it.

Referring now to Fig. 2, I indicate an area by the reference character A, and another area by the reference character B, a dotted line being drawn between the two areas and having a significance which will be brought out hereinafter. The range of alloys with which my present invention is concerned is the entire range within the irregular outline encompassing both the area A and the area B.

In my copending application above referred to, I disclose a range of composition within the ternary system manganese, iron and chromium, where hardening of the alloys could be obtained by quenching from a relatively high temperature and then reheating to an intermediate temperature, for example 500 degrees C. In that application, I offered as a working hypothesis the suggestion that hardening was due, in the range so pointed out, to the separation of finely divided alpha manganese from the ternary solid solution which had been retained at room temperature or thereabouts by the quenching operation. I now find that hardening may also take place so far as I am now able to determine by the separation of the compound FeCr.

For the purpose of simplification, I shall first consider the invention so far as it relates to alloys within the composition range marked "A." I find that the alloys within this range are all ductile at high temperatures, for example, 1200 degrees C., and remain ductile when quenched in water from that temperature. I have found that this ductility, after quenching from a high temperature, is a sharp departure in behavior between alloys made in accordance with my invention and those made with materials and methods heretofore known in the art. Quenched alloys within this composition range are magnetic and they are also unstable with regard to heat treatment at elevated temperatures, so that, on reheating to temperatures of the order of 500 degrees C. and above, a pronounced hardening action takes place.

Under appropriate conditions of composition and temperature, hardness as great as Rockwell C 60 or more may be obtained. In general, the maximum hardness is obtainable by heating for two hours at 700 degrees C. When such alloys are heated at temperatures above 700 degrees C., there is a gradually slight falling off in hardness until, at approximately 800 degrees C., the hardness begins to fall off rapidly. While all of these alloys are capable of being hardened by appropriate heat treatment, that is heat treatment appropriate to the particular composition utilized, not all of them may be given the maximum hardness possible due to the fact that some of them become so brittle as to be disrupted if they are given drastic treatment, a phenomenon which I explain as due to the separation of too great an amount of the hardening constituent.

In general, if the proportion of chromium is not above 16%, considerable if not maximum hardness may be obtained without disruption, while alloys containing somewhat more than 16%, say up to 17%, of chromium may be hardened without disruption, providing the maximum hardness which theoretically might be obtainable be not attempted. For example, alloys containing more than 16% of chromium may be appropriately hardened by quenching less drastically than in water. By quenching from 1200 degrees C. in oil, and reheating for one-half hour

at 700 degrees C., a sound alloy containing more than 10% of chromium may be produced with a hardness on the Rockwell C scale of 38. As another example, I may take a similar alloy and quench it from 1200 degrees C. in a salt bath at 500 degrees C., and obtain a hardness of Rockwell C 60. This latter alloy, however, is somewhat more brittle than the lower chromium alloys having the same hardness.

For the purpose of more fully illustrating and describing my invention, I give below a group of illustrative examples which I have made coming within the composition range A of the ternary diagram. These examples show the change of magnetism and hardness with various heat treatments and also indicate some of the results of cold work. In general, there is an increase of from 18 to 20 hardness units on the Rockwell C scale. It will be observed also that the alloys which are magnetic as quenched become non-magnetic when subsequently reheated for hardening purposes, or, in any case, the magnetism is greatly reduced by the hardening process. To the metallurgist, these changes in magnetic properties are significant so far as structure of the alloy is concerned.

#### EXAMPLE 1

##### Composition

|                             |                                                                     |                                    |    |
|-----------------------------|---------------------------------------------------------------------|------------------------------------|----|
| 30                          | Cr                                                                  | -----                              | 15 |
|                             | Mn                                                                  | -----                              | 37 |
| Balance substantially iron. |                                                                     |                                    |    |
|                             | Desulphurized with Ca.                                              |                                    |    |
|                             | Ductile as cast.                                                    |                                    |    |
| 35                          | Magnetism as cast                                                   | —0.39 g./100 g. (arbitrary units). |    |
|                             | Magnetism quenched from 1200 degrees + C.                           | —29.8 g./100 g.                    |    |
| 40                          | Magnetism heat-treated at 700 degrees C. 2 hours                    |                                    |    |
|                             | —0.80 g./100 g.                                                     |                                    |    |
|                             | Hardness quenched from 1200° + C.—C-10 (Rockwell hardness).         |                                    |    |
|                             | Hardness after severe cold work on the hammer—C-29.                 |                                    |    |
| 45                          | Hardness after heat treatment at 700° C. for 2 hours—C-60.          |                                    |    |
|                             | Heat treatments—after quenching from 1200° + C.                     |                                    |    |
| 50                          | 2 hours at 500° C.—water quench—C-45.                               |                                    |    |
|                             | 2 hours at 600° C.—water quench—C-55.                               |                                    |    |
|                             | 2 hours at 700° C.—water quench—C-60.                               |                                    |    |
|                             | ½ hour at 750° C.—water quench—C-57.                                |                                    |    |
|                             | ½ hour at 790° C.—slow cool (air)—C-58.                             |                                    |    |
| 55                          | ½ hour at 850° C.—slow cool (air)—C-38.                             |                                    |    |
|                             | Electrical resistance 85-90 micro ohms per cubed centimeter.        |                                    |    |
|                             | Coefficient of thermal expansion— $13.2 \times 10^{-6}$ cm./cm.° C. |                                    |    |

#### EXAMPLE 2

##### Composition

|                             |                                                              |    |
|-----------------------------|--------------------------------------------------------------|----|
| Cr                          | -----                                                        | 16 |
| Mn                          | -----                                                        | 32 |
| Balance substantially iron. |                                                              |    |
|                             | Notes                                                        |    |
|                             | Treated with Co—brittle as cast.                             |    |
|                             | Magnetism as cast—1.38 g./100 g.                             |    |
| 70                          | Magnetism quenched from 1200° C.—57.0 g./100 g.              |    |
|                             | Magnetism heat treated at 700° C. for 2 hours—1.68 g./100 g. |    |
|                             | Hardness as cast—C-15.                                       |    |
| 75                          | Hardness from 1200° C.—C-32.                                 |    |

Teat treatments—after quenching from 1200°  
 C. +:  
 1 hour at 700° C.—C-55.  
 ½ hour at 750° C.—water quench—C-55.  
 ½ hour at 790° C.—slow cool (air)—C-55.  
 ½ hour at 850° C.—slow cool (air)—C-41.

## EXAMPLE 3

## Composition

Cr ----- 16  
 Mn ----- 34.5  
 Balance substantially iron.

## Notes

Ductile as cast.  
 Magnetism as cast—0.35 g./100 g.  
 Magnetism quenched from 1200° C.—58 g./100 g.  
 Magnetism heat treated at 700° C. for 2 hours—  
 1.82 g./100 g.  
 Hardness quenched from 1200° C.—C-11.  
 Hardness cold worked—C-31.  
 Hardness after 700° C. heat treatment—cracked.

## EXAMPLE 4

## Composition

Cr ----- 15  
 Mn ----- 30  
 Balance substantially iron.

## Notes

Ductile as cast.  
 Magnetism as cast—4.54 g./100 g.  
 Magnetism quenched from 1200° C.—41 g./100 g.  
 Magnetism heat treated at 700° C. for 2 hours—  
 1.37 g./100 g.  
 Hardness quenched from 1200° C.—C-8.  
 Hardness after cold working—C-25.  
 Hardness after ½ hr. at 700° C.—C-47.

## EXAMPLE 5

## Composition

Cr ----- 16.5  
 Mn ----- 33  
 Balance substantially iron.

## Notes

Brittle as cast.  
 Desulphurized with Ca.  
 Non-magnetic as cast.  
 Quenched in water from 1200° C.—magnetic.  
 Quenched in furnace at 700° C. from 1200° C.,  
 1 hr. in furnace—air cool—Rb-87.  
 Oil quenched from 1200° C.—Rc-31.  
 Heated at 700° C. for ½ hr.—air cool—Rc-38.  
 Reheated to 1200° C.—water quenched—Rc-80.  
 ½ hr. at 700° C.—water quenched—Rc-30.  
 ½ hr. additional at 700° C.—water quenched—  
 —Rc-37 slight crack.  
 ½ hr. additional at 700° C. water quenched—  
 cracked.  
 Cooled on brick from 1200° C.—Rc-40.  
 Heated to 700° C. ½ hr., air cooled—Rc-40.  
 Heated to 1200° C., water quenched—cold worked.  
 Heated to 700° C., ½ hr.—cracked.  
 Quenched from 1200° C. in salt bath at 500° C.  
 for 15 minutes, air cooled, superficial Rockwell  
 C-60.

## EXAMPLE 6

## Composition

Cr ----- 18  
 Ni ----- 2  
 Mn ----- 30  
 Balance substantially iron.

## Notes

Very fine grained as cast—cannot be cold worked.  
 Hardness as cast—Rc-44.  
 Hardness annealed—Rb-96.  
 Hardness cold worked—Rc-28.  
 Hardness 500° C. Rc 26—magnetic pull 28.3.  
 Hardness 600° C. Rc 44—magnetic pull 3.44.  
 Hardness 700° C. Rc 48—magnetic pull 2.8.

10 In connection with the alloys of my present invention, particularly those of the area A, I wish to point out that their electrical resistance is relatively high and they are useful for heating elements, resistances and the like. In general, their electrical resistance is approximately the same as nichrome and other wires in current use for resistance purposes. They have the advantage of having a melting point above 1200° C. and being highly resistant to scaling up to this temperature.

15 While the properties of the alloys of my invention, and the manner in which results may be duplicated by no means require a full understanding of the hardening phenomenon, I wish to point out for the benefit of those skilled in the art by hypothesis that hardening, particularly in the case of those compounds in the area designated A, is due to a shift of the equilibrium from conditions where the phases are iron and 20 ternary solid solution to a condition where the phases are ternary solid solution and the compound FeCr. I base my hypothesis on several considerations and, in connection therewith, wish to point out that the ternary solid solution and also the compound FeCr are well known to possess stainless properties to a high degree. All of the compounds coming within the area A are capable of hardening to a very appreciable extent, and all of them possess remarkable stainless properties, at least as stainless for most purposes as the 18-8 type of so-called stainless steel which is now extensively used where higher resistance to corrosion and adequate strength are desired.

25 The alloys falling within the designated area A may be utilized with marked advantage in numerous fields. Thus, in addition to the uses referred to hereinabove, they may be employed for bearings, cutlery, machine parts where great wear resistance is required as in cams, ratchets, and the like. They may be utilized with excellent results for cooking utensils, for chemical equipment, for tools and dies, as electrodes in electrolytic operations, for relatively non-magnetic machine parts, for fabrication requiring 30 deep drawing characteristics, as thermostatic metals, for ornamental objects, and the like. They also possess the advantage of being readily welded. Their resistance to sulphur-bearing gases renders them useful for numerous purposes such as valves for automotive engines, and the like. Other uses will readily suggest themselves to those versed in the art in the light of a consideration of their various properties as herein disclosed.

35 I give separate consideration to the range indicated by the character B in the drawing, because, within this range, in my opinion, hardening takes place, for the most part, through the separation of manganese. The properties, however, are in many respects similar to the properties of the alloys in area A, although there are definite differences in the properties as well, particularly as the widely separated points in 40 the total range disclosed are reached.

Like the alloys coming within the range A, the alloys within the composition of the B range are all ductile or malleable at 1200 degrees C. and they are also malleable after quenching in water from high temperatures, such as 1100 to 1200 degrees C. They differ, however, from the alloys in the composition range A in being substantially non-magnetic in the quenched state, although here also, as well be expected, there is some gradation. They also differ from the alloys in the composition range A by undergoing a greater degree of work hardening, the increase in hardness by the cold work of the material being in general of the order of 30% on the Rockwell C scale.

The alloys in the B range may be hardened by heating after quenching in water from, for example 1200 degrees C. for short periods at 700 degrees C., or for longer periods at, for example, 500 to 600 degrees C. As a further illustration of the characteristics of these alloys, I wish to point out that they may be disrupted if heated for too long a time at temperatures of 700 degrees or thereabouts, and that this disrupting action is accentuated by quenching from such temperatures. By quenching less drastically, for example, quenching from 1200 degrees C. in a salt bath at about 500 degrees C., alloys in the B range may be obtained in a moderately hard state, but without disruption.

To further illustrate my invention, I give below four specific examples of the behavior of alloys coming within the composition range marked B. It will be noted that the range encompassed within the area marked "B" includes as one of its limiting boundaries the pure iron-manganese alloys containing from 34 to 38% iron, balance manganese with no chromium.

#### EXAMPLE 7

##### Composition

Cr----- 8  
Mn----- 50  
Balance substantially iron.

##### Notes

Ductile as cast.  
Magnetism as cast—0.11 g./100 g.  
Magnetism quenched from 1200° C. + —0.58 g./100 g.  
Magnetism quenched from 700° C. heat treatment—0.49/100 g.  
Hardness quenched from 1200° C. + —C-7.  
Hardness worked on air hammer—C-26.  
½ hour at 700° C.—slow cool—C-42.  
+ ½ hour at 700° C.—slow cool—C-42.  
Heated to 700° C.—quenched—broke up.

#### EXAMPLE 8

##### Composition

Cr----- 12  
Mn----- 50  
Balance substantially iron.

##### Notes

Can be cold worked as cast.  
Magnetism as cast—0.114 g./100 g.  
Magnetism quenched from 1100° C.—1.78 g./100 g.  
Magnetism after 2 hours at 500° C.—2.5 g./100 g.  
Magnetism after 2 hours at 600° C.—2.6 g./100 g.  
Hardness quenched from 1100 °C.—C-9.  
Hardness after 2 hours at 500° C.—C-12.  
Hardness after 2 hours at 600° C.—too brittle—disrupted.

#### EXAMPLE 9

##### Composition

Cr----- 6  
Mn----- 60  
Balance substantially iron.

##### Notes

Deforms somewhat as cast.  
Magnetism as cast—0.071.  
Magnetism quenched from 100° C. + —1.4 g./100 g.  
Magnetism after 2 hours at 500° C.—1.4 g./100 g.  
Magnetism after 2 hours at 600° C.—2.4 g./100 g.  
Magnetism after 2 hours at 700° C.—2.3 g./100 g.  
15 Hardness quenched from 1100 C. + —C-7.  
Hardness after 2 hours at 500° C.—C-14.  
Hardness after 2 hours at 600° C.—disrupted.  
Hardness after 2 hours at 700° C.—disrupted.

#### EXAMPLE 10

##### Composition

Cr----- 8.5  
Mn----- 50

##### Notes

Quenched in salt bath at 500° C. from 1200° C.—15 minutes at 500° C.—air cooled—Hardness, Rockwell B-73.  
30 Heated ½ hr. at 600° C. in salt bath, air cooled (does not ring), Rc-24.  
Heated ½ hr. at 700° C. in salt bath—Rc- 24.  
Heated 1 hr. additional at 700° C., air cooled.

The alloys encompassed within the area B may also be employed for a multitude of purposes as, for example, cams, ratchets, and machine parts where great wear is required, for fabrication purposes requiring great ductility, for parts requiring resistance to sulphur-bearing gases, and the like.

An examination of my co-pending application will show that I disclose therein an alloy consisting of 36% iron and 64% manganese having properties similar to those of the iron-chromium and manganese alloys and the character of the curves shown in the drawing indicates clearly the relationship of this alloy to the other alloys within the scope of the present invention. It appears, therefore, that hardenable manganese alloys have a definite relationship to the hardenable iron-chromium manganese alloys. As an illustration, the alloy noted, namely the alloy of 36% iron, remainder manganese, is ductile and non-magnetic as quenched from 1100 degrees C. 55 Its Rockwell hardness in this condition is approximately C-3. On cold working, its hardness increases to approximately C-35, and by heating the quenched alloy for thirty minutes at 600 degrees C., its hardness becomes approximately C-56. These figures are illustrative of the results obtained on relatively large numbers of samples.

In my prior copending application above referred to, I disclose the desirable effects of the additions of small amounts of nickel, copper, and titanium, and such substances, to alloys of iron, manganese and chromium. It should be understood that small amounts of these and other elements including carbon may be added to the alloy compositions which I have disclosed without departing from the practice of my invention. By the addition of such carbon as is introduced by employing calcium carbide as a desulphurizer, the hardening of the alloys in Region A is, how-

ever, considerably lessened with some increase in ductility. While I prefer to employ pure manganese of the character identified, certain phases of my invention may be practiced with fair results by the use of manganese containing not substantially more than 1.0% of other materials. I have found, however, that markedly superior results are obtained with substantially pure manganese and its use is definitely preferred. Such substantially pure manganese is preferably electrolytic manganese, desulphurized preferably by the use of metallic calcium.

It will be appreciated that the chromium and iron utilized in the alloys should be of sufficient purity so as not to introduce deleterious amounts of other metals. Those versed in the art will, in the light of my teachings herein, readily be able to choose chromium and iron of sufficient purity to accomplish the production of alloys fulfilling the objects of my invention.

Thus it will be seen that I have discovered improved alloys of manganese, iron and chromium, the constitution of which may be determined by reference to the irregular area outlined in the drawing. Thus the chromium content may run up to 17% or slightly above, the manganese may range between approximately 25% and 65%, and the iron between about 43 and 67%. While these extreme ranges may be modified slightly, in general it will be found that such modification will be at the expense of desirable properties. In the range, approximately 11.5 to 16% chromium and up to even 17.5% chromium, following suitable precautions, with from approximately 25% to 43% manganese and 43% to 58% iron, a particu- 35

larly desirable combination of properties is obtained, including extreme hardness where desired, more than adequate ductility and malleability for working, and unusual resistance to corrosion. This range is, as before noted, in the general area marked with reference character A. As we move down toward the lower right hand portion of the indicated area, particularly where we pass the region shown by the dotted lines, the properties show variation, particularly in some loss of resistance to corrosion, with a concomitant decrease in hardening by heat treatment but with an increase in work hardening.

From the description of the alloys of my invention, those skilled in the art will understand at once the large number of uses to which they may be applied. It is sufficient to point out that the industrial uses are almost unlimited where hardened stainless alloys are required. These are uses to which alloys of the same general type, that is to say, stainless alloys hardened without the use of carbon, have so far as I know never been applied before.

What I claim as new and desire to protect by Letters Patent of the United States is:

Alloys hardenable without cracking by heating, cooling and reheating to a lower temperature, said alloys consisting essentially of chromium, manganese and iron in the following proportions: from 6% to 12% chromium, from 50% to 60% manganese, and the balance iron, with the exception of such small amounts of impurities as will not affect the properties of the alloys.

REGINALD S. DEAN.